

May 23, 1950

D. A. NEWMAN

2,508,725

TRANSFER MEDIUM

Filed Jan. 13, 1945

*Fig. 1*



*Fig. 2*



*Fig. 4*



*Fig. 5*



INVENTOR  
Douglas A. Newman  
BY *Johnson + Kline*  
ATTORNEYS

## UNITED STATES PATENT OFFICE

2,508,725

## TRANSFER MEDIUM

Douglas A. Newman, Port Washington, N. Y., assignor to Columbia Ribbon and Carbon Manufacturing Company, Inc., Glen Cove, N. Y., a corporation of New York

Application January 13, 1945, Serial No. 572,698

9 Claims. (Cl. 282--28)

1

This invention relates to transfer sheets and to the method of making the same.

Such sheets have a suitable foundation carrying a pigmented coating and are used sometimes to transfer inscriptions or images made on or over them to another sheet, as, for instance, in making "carbon" copies, or hectograph master-sheets for subsequent transfer to a gelatine sheet or blank or directly to a printing sheet if the spirit method of duplication is to be used. For sharp clear impressions, it has been found that the more homogeneous the foundation sheet and the smoother the coated surface the better the results. Sheets molded or formed of plastic compounds have these desired characteristics.

In some cases, the transfer sheet is to be used as a slide or transparency for transferring by light rays the inscriptions or images thereon to a screen. In the latter case, the body or foundation of the sheet should be as transparent as possible. Here again, sheets molded or formed of plastic compounds, which may be transparent or translucent, of which cellulose-acetate sheets and "cellophane" are examples, are ideally suitable.

It is a desideratum that coating on the sheet be loose-bonded so that substantially all of the pigmented coating is transferable to the master sheet if for hectography, or from the transfer sheet if it is to be used as a transparency. Yet, for either use, the coating should cling to the sheet against cracking or flaking off in ordinary handling or flexing, and should only transfer under the pressure forming the images or inscriptions.

The difficulties of meeting these contrary requirements have been aggravated by the smoothness and lack of tooth of the preferred foundation of such sheet, i. e., "cellophane."

These difficulties have been overcome by the present invention by providing between the sheet of "cellophane" and the pigmented transferable coating, a bonding coating which has the ability to adhere to the smooth-surfaced, substantially non-impregnable plastic-body sheet and at the same time itself provide a moderately toothed surface to which the transferable coating may cling until, by the application of pressure, as in writing, drawing with a stylus, typewriting or printing from type, it is forcibly transferred to another medium.

By varying the composition of the bonding coating, its tenacity for the pigmented coating may be varied so that varying degrees of pressure are required to transfer it from the bonding coating.

2

Preferably, however, the bonding coating has greater affinity for, or adhesion to, the "cellophane" surface than to the pigmented coating, so that it may be left behind on the foundation when the ink is transferred. When the foundation is to be used as a transparency, it is preferable that the bonding coating itself be transparent, or at least translucent, and it may be colorless. However, if the projected image is to be in colored light, the bonding coating, according to the present invention, may be tinted for that purpose.

At present, it is advantageous to use, as a bonding layer, a coating including a Vinylite resin of the polyvinyl butyral series, for it has been found that this is highly receptive to ink and carbon coatings, is non-absorptive of, and insoluble by, the hot or molten ink and carbon coating compositions. Other suitable bonding coatings may, however, be used within the spirit of this invention.

Other features and advantages will hereinafter appear.

Referring to the drawing:

Figure 1 is a view of the transfer sheet of the present invention.

Fig. 2 is a view of a portion of the transfer sheet showing the clear places left when the pigmented coating is transferred therefrom to another medium.

Fig. 3 is a magnified sectional view taken on the line 3—3 of Fig. 2.

Fig. 4 is a magnified sectional view of a portion of the transfer sheet of the present invention, showing in approximate proportion the relative thickness of the foundation, the bonding coating, and the transferable coating.

Fig. 5 is a view of the transfer sheet of the present invention as made and used in the form of a continuous strip or ribbon.

The foundation 10 of the transfer sheet of the present invention is molded or formed of a solidified resin, synthetic resin, or other similar or substitute material, to be substantially homogeneous, smooth-surfaced, and substantially non-porous, and which will, in sheets of such thicknesses as are practically employed for the purposes herein intended, be tough, strong, flexible and non-plastic at temperatures in which it may be used. By way of example, it may be mentioned that cellulose acetate sheets and the product commercially known as "cellophane" have such properties and have been satisfactorily used in practicing this invention.

Because it is substantially non-absorptive and smooth-surfaced, such a foundation, when coated with a transferable pigmented coating, must be

handled with extreme care both in manufacture and before and during its use, because the coating adheres to the smooth surface of the foundation with so little tenacity that the slightest abrading or rubbing action or pressure on the sheet will cause the coating to be transferred off the sheet either onto the surface causing the transfer, or to an adjacent medium; also, in use, the flexing of the sheet, such as caused by introducing it to and wrapping it around the platen of a typewriter, causes the pigmented coating to check or flake off.

The voids produced by the scratched or flaked-off portions of the coating, if coinciding with impressions or inscriptions desired to be made, result in faulty and unsatisfactory images being produced on the master sheet and reproduced on the worksheets. If, while the master sheet and transfer sheet are against each other, for instance while being assembled, introduced to the platen, fed around the same, or removed from the typewriter, the particles of the transferable coating are flaked off, it is probable that they will lodge upon the master sheet and be reproduced on the worksheet as objectionable, or to say the least, undesirable background.

To overcome these difficulties, the present invention provides on the surface of the foundation 10 which is to be coated, a coating or layer 11 which will adhere or cohere to the smooth surface of the foundation and itself provide a surface having sufficient tooth to anchor and hold the pigmented transferable coating.

After the bonding coating 11 has been applied to the foundation 10, the strip is coated with molten, or at least hot, transfer ink to produce the transferable coating 12 which adheres to the toothed surface of the bonding coating with sufficient tenacity to remain attached in normal handling and use and yet be substantially all transferred to a master sheet against which the coating is placed upon the application of printing or writing pressure. By varying the composition of the bonding coating, the adhesion of the transfer coating thereto may be increased to a point where only a predetermined amount of pressure will cause it to transfer.

It has been found that excellent results are obtained when the bonding coating comprises a vinylite resin of the polyvinyl butyral series, a solvent and plasticizer, for the coating formed thereby is flexible and tough and adheres firmly to the foundation, and provides the desired amount of toothed surface for receiving the transfer ink coating. It is stable and not soluble in the molten or hot wax or oil of the transfer ink.

If desired, a small amount of filler may be added to the coating compound to provide greater tooth to the coating for obtaining greater adhesion of the transfer material to the bonding coating, especially when the transfer material is hectographic ink. Fillers such as colloidal clay, barium sulphate, and titanox have been satisfactory.

When the transfer sheet is to be used as a transparency to light ray projection, the fillers should be dispensed with, and if it is desired to have the image appear in colored light, a dye or other coloring material may be incorporated in the bonding coating 11.

As stated above, the affinity of the bonding coating 11 for the foundation 10 is greater than its affinity for the transferable coating, and hence, when the transfer takes place, the coating 11 remains behind on the foundation and the

pigmented coating 12 transfers and adheres to the master sheet to be yielded up to the gelatine pad or blanket or directly to the worksheets if used in a spirit duplicator.

It has been found that a foundation .002 inch thick, and bonding coating .002 inch thick, and a pigmented coating .003 inch thick give excellent results. These dimensions are given by way of example and are not to be construed as limiting the invention in any way whatsoever.

The product of the present invention may be used in the form of a sheet as shown in Fig. 1, or as a continuous strip or ribbon 13 as shown in Fig. 5.

Variations and modifications may be made within the scope of this invention and portions of the improvements may be used without others.

I claim:

1. A transfer element comprising a foundation of homogeneous flexible material having a smooth non-porous working surface; a bonding coating tenaciously adhering to said working surface; and a pigmented coating consisting essentially of high melting point wax, oils and coloring matter releasably adhering to said bonding coating, the adhesion between the pigmented coating and the bonding coating being such as to permit the former to transfer substantially entirely to another medium under printing or writing pressure, and the adhesion between the bonding coating and the foundation being such that the bonding coating remains on the foundation upon printing or writing pressure causing transfer of the pigmented coating, said bonding coating consisting essentially of a resinous material which is substantially insoluble in the hot oil and wax of the pigmented coating when molten.

2. A transfer element comprising a foundation of thin, light, tough, flexible, homogeneous, translucent material having a smooth non-porous working surface; a thin, flexible bonding coating tenaciously adhering to said working surface; and a pigmented coating consisting essentially of high melting point wax, oils and coloring matter releasably adhering to said bonding coating, the adhesion between the pigmented coating and the bonding coating being such as to permit the former to transfer substantially entirely to another medium under printing or writing pressure, and the adhesion between the bonding coating and the foundation being such that the bonding coating remains on the foundation upon printing or writing pressure causing transfer of the pigmented coating, said bonding coating consisting essentially of a translucent resinous material which is substantially insoluble in the hot oil and wax of the pigmented coating when molten.

3. A transfer sheet or strip comprising a foundation of thin cellulosic film, a thin flexible bonding coating of vinylite resin tenaciously adhering to the working surface of the foundation, and a pigmented transfer coating releasably adhering to said bonding coating, the adhesion between the pigmented coating and the bonding coating being such as to permit the former to transfer substantially entirely to another medium under printing or writing pressure, and the adhesion between the bonding coating and foundation being such that the bonding coating remains on the foundation upon printing or writing pressure causing transfer of the pigmented coating.

4. A transfer sheet or strip comprising a foundation of thin cellulosic film, a thin flexible bonding coating of vinylite resin tenaciously adhering to the working surface of the foundation, and a transferable high melting point wax, pigmented

75

coating releasably adhering to said bonding coating, the adhesion between the pigmented coating and the bonding coating being such as to permit the former to transfer substantially entirely to another medium under printing or writing pressure, and the adhesion between the bonding coating and the foundation being such that the bonding coating remains on the foundation upon printing or writing pressure causing transfer of the pigmented coating.

5. A transfer sheet or strip comprising a foundation of thin cellulosic film, a thin flexible bonding coating of a solidified polyvinyl butyral compound tenaciously adhering to the working surface of the foundation, and a pigmented transfer coating releasably adhering to said bonding coating, the adhesion between the pigmented coating and the bonding coating being such as to permit the former to transfer substantially entirely to another medium under printing or writing pressure, and the adhesion between the bonding coating and foundation being such that the bonding coating remains on the foundation upon printing or writing pressure causing transfer of the pigmented coating.

6. A transfer sheet or strip comprising a foundation of thin cellulosic film, a thin flexible bonding coating of a solidified polyvinyl butyral compound including a filler tenaciously adhering to the working surface of the foundation, and a pigmented transfer coating releasably adhering to said bonding coating, the adhesion between the pigmented coating and the bonding coating being such as to permit the former to transfer substantially entirely to another medium under printing or writing pressure, and the adhesion between the bonding coating and foundation being such that the bonding coating remains on the foundation under printing or writing pressure causing transfer of the pigmented coating.

7. A transfer sheet or strip comprising a foundation of homogeneous flexible material having a smooth non-porous working surface, a thin flexible bonding coating of vinylite resin tenaciously adhering to the working surface of the foundation, and a pigmented transfer coating releasably adhering to said bonding coating, the adhesion between the pigmented coating and the bonding coating being such as to permit the former to transfer substantially entirely to another medium under printing or writing pressure.

and the adhesion between the bonding coating and the foundation being such that the bonding coating remains on the foundation upon printing or writing pressure causing transfer of the pigmented coating.

8. A transfer sheet or strip comprising a foundation of homogeneous flexible material having a smooth non-porous working surface, a thin flexible bonding coating of vinylite resin tenaciously 10 adhering to the working surface of the foundation, and a transferable layer having a high melting point, pigmented wax coating releasably adhering to said bonding coating, the adhesion between the pigmented coating and the bonding 15 coating being such as to permit the former to transfer substantially entirely to another medium under printing or writing pressure, and the adhesion between the bonding coating and the foundation being such that the bonding coating remains on the foundation upon printing or writing 20 pressure causing transfer of the pigmented coating.

25 9. A transfer sheet or strip comprising a foundation of homogeneous flexible material having a smooth non-porous working surface, a thin flexible bonding coating of a solidified polyvinyl butyral compound tenaciously adhering to the working surface of the foundation, and a transferable layer having a high melting point, pigmented 30 wax coating releasably adhering to said bonding coating, the adhesion between the pigmented coating and the bonding coating being such as to permit the former to transfer substantially entirely to another medium under printing or writing pressure, and the adhesion between the bonding coating and the foundation being such 35 that the bonding coating remains on the foundation upon printing or writing pressure causing transfer of the pigmented coating.

DOUGLAS A. NEWMAN.

#### REFERENCES CITED

The following references are of record in the file of this patent:

UNITED STATES PATENTS

| Number    | Name                 | Date           |
|-----------|----------------------|----------------|
| 1,925,235 | Dixon -----          | Sept. 5, 1933  |
| 1,929,601 | Miner -----          | Oct. 10, 1933  |
| 2,357,948 | Gessler et al. ----- | Sept. 12, 1944 |
| 2,372,209 | Kohler -----         | Mar. 27, 1945  |